



US006675838B2

(12) **United States Patent**  
**Arthurs et al.**

(10) **Patent No.:** **US 6,675,838 B2**  
(b4) **Date of Patent:** **Jan. 13, 2004**

(54) **ANTI-STATIC WOVEN FABRIC AND FLEXIBLE BULK CONTAINER**(75) Inventors: **Trevor Arthurs**, Truro (CA); **W. Keith Fisher**, Suffield, CT (US)(73) Assignees: **IPG Technologies, Inc.**, Columbia, SC (US); **S lutia, Inc.**, Cantonment, FL (US)

(\*) Notice: Subject to any disclaimer, the term of this patent is extended or adjusted under 35 U.S.C. 154(b) by 131 days.

(21) Appl. No.: **10/003,890**(22) Filed: **Oct. 25, 2001**(65) **Prior Publication Data**

US 2002/0129864 A1 Sep. 19, 2002

**Related U.S. Application Data**

(60) Provisional application No. 60/242,999, filed on Oct. 25, 2000.

(51) **Int. Cl.<sup>7</sup>** ..... **D03D 15/00**(52) **U.S. Cl.** ..... **139/420 A**; 139/420 R; 139/426 R; 383/24; 383/117; 442/189(58) **Field of Search** ..... 139/420 R, 420 A, 139/426 R; 428/244, 245, 255, 257, 258, 265, 297; 383/24, 117; 442/189, 197(56) **References Cited****U.S. PATENT DOCUMENTS**

- |             |   |         |        |         |
|-------------|---|---------|--------|---------|
| 3,639,528 A | * | 2/1972  | Patton | 525/203 |
| 3,803,453 A | * | 4/1974  | Hull   | 361/220 |
| 4,422,483 A |   | 12/1983 | Zins   |         |
| 4,431,316 A |   | 2/1984  | Massey |         |

|                 |         |                     |           |
|-----------------|---------|---------------------|-----------|
| 4,606,968 A     | 8/1986  | Thornton et al.     |           |
| 4,753,088 A     | 6/1988  | Harrison et al.     |           |
| 4,856,299 A     | 8/1989  | Bryant              |           |
| 5,071,699 A     | 12/1991 | Pappas et al.       |           |
| 5,167,264 A     | *       | 12/1992 Kalin ..... | 139/420 R |
| 5,288,544 A     | 2/1994  | Mallen et al.       |           |
| 5,478,154 A     | 12/1995 | Pappas et al.       |           |
| 5,512,355 A     | 4/1996  | Fuson               |           |
| 5,679,449 A     | 10/1997 | Ebadat et al.       |           |
| 6,057,032 A     | 5/2000  | Green               |           |
| 6,112,772 A     | 9/2000  | Ebadat et al.       |           |
| 6,287,689 B1    | 9/2001  | Elliott et al.      |           |
| 6,413,635 B1    | 7/2002  | Martin et al.       |           |
| 6,451,407 B1    | 9/2002  | Nickell             |           |
| 2002/0136859 A1 | 9/2002  | Fisher et al.       |           |

**OTHER PUBLICATIONS**

U.S. patent application Ser. No. 60/137,615, Fisher et al., filed Jun. 3, 1999.

\* cited by examiner

*Primary Examiner*—John J. Calvert*Assistant Examiner*—Robert H. Muromoto, Jr.(74) *Attorney, Agent, or Firm*—Roberts Abokhair & Mardula, LLC(57) **ABSTRACT**

A method of making an ungrounded type flexible fabric container with a reduced energy of electrostatic discharge for use in a combustible environment is provided. A woven fabric is configured to form a flexible fabric container having sidewalls, a closed end and an open end. The woven fabric made as from a static dissipating fabric comprising fabric woven of non-conductive tapes, to which a plurality of conductive staple fibers are woven into or coated onto the fabric at a spacing of from 3 mm to 100 mm.

**23 Claims, 1 Drawing Sheet**



Figure 1

## ANTI-STATIC WOVEN FABRIC AND FLEXIBLE BULK CONTAINER

### CROSS REFERENCE TO OTHER PATENT APPLICATIONS

This application claims priority under 35 U.S.C. 119 from U.S. provisional patent application Ser. No. 60/242,999 filed Oct. 25, 2000 of the same title and inventors, which is incorporated by reference in its entirety.

### BACKGROUND OF THE INVENTION

In the past, various methods have been employed to produce anti-static woven fabrics suitable for flexible intermediate bulk containers (FIBC) or clean room garments. FIBCs are used in the packaging and transportation of dry substances such as metal ores, chemicals, foodstuffs and powders. They are designed to be handled with standard fork-lifts and typically hold from 500 to 4400 pounds of material. Common dimensions include 35 inch and 41 inch square cylinders. A common hazard of FIBCs is electrostatic discharge (ESD). ESD hazard ranges from personnel nuisance shocks to sparks capable of igniting explosive mixtures of dust or flammable gases. As a result it is necessary to eliminate ESD from flexible intermediate bulk containers in certain applications.

Clean room garments are worn by operators working in clean room environments, typically for the manufacture of semi-conductor electronic components. Often the semi-conductors are sensitive to electrostatic discharges and are damaged when subjected to ESD. The result is that clean room garments must in many cases be free of ESD, just as FIBCs must be.

Some of the textile fabrics used in FIBC and clean room garments include polypropylene and Tyvek®. Polypropylene is particularly favored for FIBCs due to its inertness, strength and low cost. FIBCs made from woven polypropylene are disclosed in U.S. Pat. No. 5,071,699 to Pappas that is incorporated by reference herein.

FIBCs are either coated or uncoated. Uncoated FIBCs are breathable and allow transmission of moisture through the fabric. Coated FIBCs can restrict transmission of moisture; prevent dust escaping as well as having other special properties. For example, when ultraviolet light resistance is desired, a UV stabilizing coating is used. As an alternate, threads and yarns can be coated with a UV stabilizer before weaving into fabric.

Control of ESD from fabrics can be either conductive or dissipative. Conductive refers to the electrical conduction of any accumulated charge, to an electrical ground. Dissipative refers to the dissipation of static electricity through electrostatic discharges including corona discharges, spark discharges, brush discharges or propagating brush discharges. Spark, brush and propagating brush discharges can create incendiary discharges in many common flammable atmospheres. In contrast the corona discharges are generally below incendiary discharge energy levels.

Conductive fabrics require an electrically sufficient connection to a ground point. These fabrics function by draining an accumulating electrical charge to the ground. Any disruption in the ground connection disables their ESD control ability. Additionally, fabrication of containers formed of conductive fabrics requires specialized construction techniques to ensure all conductive surfaces are electrically connected together for a ground source.

In contrast, dissipative fabrics rely on the fabric, alone or in conjunction with an anti-static coating, to discharge

charges at levels below those that cause damage or create a spark capable of igniting flammable material (for example by corona discharge). Examples of dissipative fabrics are disclosed in U.S. Pat. No. 5,512,355 to Fuson and assigned to E. I du Pont and U.S. Patents assigned to Linq Industrial Fabrics, including U.S. Pat. No. 5,478,154 to Pappas et al, U.S. Pat. No. 5,679,449 to Ebadat et al., U.S. Pat. No. 6,112,772 to Ebadat et al.

The fabrics disclosed in U.S. Pat. No. 5,512,355 comprise polypropylene yarns interwoven with sheath-core filament yarns. The sheath-core filament yarns further comprise semi-conductor carbon black or graphite containing core and a non-conducting sheath. The filaments are interlaced in the fabric at between  $\frac{1}{4}$  and 2 inch intervals. In a preferred embodiment, the filaments are crimped so that stretching of the sheath-core yarn does not break the electrical continuity of the semi-conductor core. A noted disadvantage of sheath-core filaments is the relatively high cost of resultant yarns.

The fabrics disclosed (but not claimed) in the Linq Industries assigned patents also comprise sheath-core yarns interwoven with non-conductive yarns or superimposed over non-conductive yarns. Such fabrics are identified as "quasi-conductive," conduct electricity through the fabric and have surface resistivity of  $10^9$  to  $10^{12}$  ohms per square and the sheath-core yarns are identified as "quasi-conductive" with a resistance of  $10^8$  ohms per meter. In order to attain the disclosed surface resistivity an antistatic coating is utilized. Without antistatic coating, the sheath-core yarns must be placed at a narrow spacing with the effective discharge area between the sheath-core yarns limited to 9 mm.

These patents teach against the use of conductive fibers in ungrounded antistatic applications. When relying upon the sheath-core yarns for static dissipation these fabrics are costly. In contrast, when relying on antistatic coating alone, such fabrics are susceptible to failure if the coating becomes removed during use. Additionally, when FIBCs comprise such fabrics are filled with non-conductive powders a surface charge potential of -32 kV (negative 32 kV) can be attained.

U.S. Pat. No. 5,071,699 to Pappas et al. discloses the use of conductive fibers in ungrounded antistatic fabric further comprising an antistatic coating. The resultant surface resistivity of the fabric is 1.75 times  $10^{13}$  to 9.46 times  $10^{13}$ . When the coating is not present the disclosed fabrics do not adequately dissipate static charges. As a result, care must be taken to preserve the integrity of the coating.

The above patents are incorporated by reference. It is seen from the above that what is needed is a dissipative antistatic fabric that does not rely upon antistatic coatings or sheath-core filament yarns.

As a result, it is seen that a more robust anti-static textile fabric capable of preventing high surface charge levels is desirable, particularly a fabric that does not rely upon anti-static coatings or narrow spacing of quasi-conductor yarns.

### BRIEF SUMMARY OF THE INVENTION

In one embodiment, the present invention comprises a fabric with reduced electrostatic discharge energy suitable for ungrounded use in combustible atmospheres, clean room environments and flexible fabric containers. In some embodiments of the present invention, flexible fabric containers are constructed of the fabric and have reduced surface charge during filling operations of flexible fabric containers. The static dissipating fabrics of the present

invention comprise fabric woven of non-conductive tapes, to which a plurality of conductive staple fibers are woven into or coated onto the fabric at a spacing of from 3 mm to 100 mm.

#### BRIEF DESCRIPTION OF THE DRAWINGS

FIG. 1 schematically illustrates one embodiment of the invention.

#### DETAILED DESCRIPTION OF THE INVENTION

The present invention relates to the method of producing anti-static fabric suitable for use in ungrounded flexible intermediate bulk containers (FIBC) and clean room garments. FIG. 1 shows a representative cross-sectional view of such a fabric. The fabric generally designated as 1 comprises a non-conductive fabric of non-conductive tapes 2 and 4 into which a staple yarn 3 comprised of conducting segments is woven in either the weft or warp directions. In one embodiment the staple yarn is woven in the weft direction at intervals from 3 mm to 100 mm. When used as a fabric for flexible intermediate bulk containers (FIBC) the interval is preferably from 10 mm to 100 mm, and more preferably 25 mm. When used as a fabric for clean room garments, the interval is preferably 3 mm to 25 mm.

At greater intervals for the staple yarn, less corona discharge points are available. At distances greater than about 100 mm, the antistatic properties of the fabric become limited and reliance on antistatic coating effects is requisite. At very short intervals the antistatic properties are superior. However, at short intervals the cost and difficulty of manufacture increases. A good balance between needed antistatic property and cost is achieved at a 25 mm interval for fabric to be utilized in FIBCs.

The non-conductive tapes 2 and 4 of FIG. 1 may be any suitable non-conductive tapes. One embodiment of the invention comprises polypropylene non-conductive tapes. Common polypropylene tapes of 500 to 4000 denier and width of 1.7 mm to 10 mm are suitable. Polypropylene tapes narrower than 1.7 mm are often too thick and brittle for weaving into the fabric. Similarly polypropylene tapes wider than 10 mm are typically too thin and frequently break during weaving.

The staple yarn 3 of FIG. 1 may comprise any suitable conductive staple yarn with carbon loaded conductive polymer paths on the surface of the yarn. For example, suitable yarns are available from Solutia Inc. as No Shock® yarns. For example, No-Shock® 285-E3S yarn is such a suitable yarn.

Manufacture of staple yarn is known in the art and consists of spinning multiple short lengths of fibers together. For example, a staple yarn may contain fibers of a consistent 1.5 inch length that are spun together into a single multi-fiber yarn. In such yarns, each staple length is separate from each other length with only casual mechanical contact between lengths. As a result, when the staple lengths are further comprised of conductor or semi-conductor fibers, electrical discontinuity exists between staple lengths.

Surprisingly, it has been determined that the electrical discontinuity enhances the ability of the yarn to control electrostatic charge densities in an ungrounded fabric. It is thought that the shorter conductor segments limit the capacitance of the yarn thereby reducing charge density. In addition, the numerous sites of electrical discontinuity provide greater numbers of corona discharge sites than methods

heretofore disclosed. As a result, superior anti-static performance is accomplished with fabric comprising such yarns. Similarly, fabrics with equivalent anti-static performance are produced from lesser amounts of conducting yarn or with 5 yarn at a wider spacing.

Surprisingly when fabrics are produced incorporating such yarn, they are capable of dissipating electrical static charges without the use of anti-static coatings.

The invention is illustrated, but not limited by the following examples:

#### EXAMPLES AND PREFERRED EMBODIMENTS

Tests were performed on FIBCs sewn of fabrics comprised of three different conductive staple yarns woven into a non-conductive 6.5 ounce fabric at intervals of 1 inch. Conductive staple yarn designated as yarn #1 comprise an antistatic yarn consisting of a core of continuous conductive fibers surrounded by a sheath of staple fibers produced via standard core spinning techniques. Equal portions by weight of core continuous fibers and sheath staple fibers are used. The core continuous conductive fibers are bicomponent fibers consisting of a sheath of conductive polymer (nylon 6,6 loaded with about 30% weight carbon) completely surrounding a core of non-conductive nylon. The total denier of the formed antistatic yarn is 616.

Conductive staple yarn designated as yarn #2 comprise an antistatic yarn consisting of 50% weight conductive staple fibers and 50% weight non-conductive fibers produced via 30 standard ring-spinning techniques. The conductive staple fibers are obtained starting from an 18 denier, 2 continuous fiber yarn, wherein each filament is a bicomponent conductive "racing stripe" fiber having 3 longitudinal stripes of a carbon loaded conductive constituent on the surface of a 35 non-conductive nylon constituent (No-Shock® 18-2E3N yarn from Solutia, Inc.) This starting material is twice drawn to 4.5 denier per filament, then cut to a fiber length of 1.5 inches and ring spun with non-conductive nylon staple fibers (2.1 denier per filament, 1.5 inch fiber length). The total 40 denier of the formed antistatic yarn is 471.

Conductive staple yarn designated as yarn #3 comprise an antistatic yarn consisting of a core of continuous conductive fibers surrounded by a sheath of conductive staple fibers is 45 produced via a standard DREF core spinning technique. Equal portions by weight of core continuous fibers and sheath staple fibers are used. The core continuous conductive fibers are bicomponent fibers consisting of a sheath of 50 conductive polymer (nylon 6,6 loaded with about 30% weight carbon) completely surrounding a core of non-conductive nylon. The surrounding conductive staple fibers are the same twice-drawn 4.5 denier per filament, 3-“racing stripe” fibers described in yarn #2. The total denier of the 55 formed antistatic yarn is 632.

Table 1 indicates results obtained during incendivity testing of FIBCs sewn from fabrics comprising the three different conductive staple yarns. The three sample fabrics and the compare fabric included antistatic yarn woven into the fabric at an interval of about 25 mm. Sample 1 included 60 comprised yarn #1, sample 2 comprised yarn #2 and sample #3 comprised yarn #3. Compare fabric comprised yarn formed from continuous lengths of the antistatic fibers of yarns #1, #2 and #3.

Testing indicates that when the fabric comprises continuous conductive yarn as opposed to staple conductive yarn the fabric fails the incendivity test. Of importance is the external nature of the antistatic yarn. Yarns of both conduc-

tive and non-conductive cores performed properly when the exterior comprised staple yarn segments. Such incendivity testing demonstrates the reduced energy nature of the corona discharges that are below incendiary discharge energy levels.

TABLE 1

| Sample                  | Discharge Incendivity Test<br>(4.4% Propane in Air, Ignitions occur at 0.24 to 0.25 mJoules) |                                    |                                                    |                                                |
|-------------------------|----------------------------------------------------------------------------------------------|------------------------------------|----------------------------------------------------|------------------------------------------------|
|                         | Number of Ignitions (Ambient Humidity)                                                       | Number of Ignitions (Low Humidity) | Mean Max. Surface Potential (kV, Ambient Humidity) | Mean Max. Surface Potential (kV, Low Humidity) |
| 1                       | 0 of 100 tests                                                                               | 0 of 100 tests                     | -10                                                | -10.9                                          |
| 2                       | 0 of 100 tests                                                                               | 0 of 100 tests                     | -11.5                                              | -10.9                                          |
| 3                       | 0 of 100 tests                                                                               | 0 of 100 tests                     | -8.5                                               | -11.1                                          |
| Compare Fabric Standard | 99 of 100 tests                                                                              | 99 of 100 tests                    | -37.3                                              | -37.8                                          |
| FIBC                    | 100 of 100 tests                                                                             | 100 of 100 tests                   | -57.3                                              | -53.1                                          |

For testing, each FIBC was filled with a test powder, polypropylene pellets, at a rate of one kilogram per second and in accordance with procedures in the reference document "Testing the Suitability of FIBCs for Use in Flammable Atmospheres", Vol 15, No. 3, 1996 AIChE. As seen in Table 1, all three FIBCs comprising antistatic fabrics of the present invention passed incendiary testing. Noteworthy is the low surface potential produced in these fabrics as compared to standard polypropylene FIBC or FIBCs comprised of compare fabrics.

When fabrics are used in FIBCs, it is common to coat the fabrics for improved retention of contents as well as resistance to ultraviolet light and other atmospheric oxidants. An example of a preferred coating is:

1.0 mil coating further comprised of:  
 73.5% polypropylene homopolymer  
 19% low density polyethylene  
 1.5% Ultraviolet Light absorbers (for example MB176 available from Synergistics)  
 6% of a dilute antistatic coating (for example AS6437B available from Polymer Products)

Surprisingly it has been determined that the antistatic coating, although helpful, is not essential to the adequate antistatic performance of the fabric. As a result, sufficient antistatic performance is present after instances of coating failure. Examples of causes of coating failures include abrasive wear, chemical, ultraviolet and other environmental causes.

Further testing confirmed that the fabrics of the present invention prevent incendiary discharges without the presence of antistatic coating. In a more rigorous testing of antistatic performance, sample fabric #1 was first coated with a 1 mil coating comprising:

79.5% polypropylene homopolymer  
 19% low density polyethylene  
 1.5% Ultraviolet Light absorbers (for example MB176 available from Synergistics)

This fabric was then tested in an ethylene atmosphere capable of ignition at 0.07 mJoules (as opposed to 0.24–0.25 mJoules of Table 1). No incendiary discharges were observed after 100 tests. This demonstrates that the need for expensive antistatic coatings are eliminated in the present invention.

Another preferred embodiment of the invention is 3.0 ounce rated fabric comprising fabric woven of non-conductive tapes, to which a plurality of conductive staple fibers are woven or coated into the fabric at a spacing of from 3 mm to 100 mm, preferably at a spacing from 10 mm to 100 mm, and most preferably at a spacing of 25 mm. The non-conductive tapes form a polypropylene fabric further comprising 11 of 900 denier tapes/inch in the warp direction and 9 of 1300 denier tapes/inch in the weft direction. The tapes further comprise polypropylene homopolymer with ultraviolet inhibitors. Coatings may be applied to the fabric to improve content retention and moisture exclusion properties. One embodiment of the invention uses a coating comprising 73.5% weight polypropylene homopolymer; 19% weight low density polyethylene polymer; 1.5% weight ultraviolet inhibitors and 6% weight of 25% weight antistatic masterbatch.

One embodiment of the invention is 6.5 ounce rated fabric comprising fabric woven of non-conductive tapes, to which a plurality of conductive staple fibers are woven or coated into the fabric at a spacing of from 3 mm to 100 mm, preferably at a spacing from 10 mm to 100 mm, and most preferably at a spacing of 25 mm. The non-conductive tapes form a polypropylene fabric further comprising 16 of 1600 denier tapes/inch in the warp direction and 12 of 2300 denier tapes/inch in the weft direction. The tapes further comprise polypropylene homopolymer with ultraviolet inhibitors. Coatings may be applied to the fabric to improve content retention and moisture exclusion properties. One embodiment of the invention uses a coating comprising 73.5% weight polypropylene homopolymer; 19% weight low density polyethylene polymer; 1.5% weight ultraviolet inhibitors and 6% weight of 25% weight antistatic masterbatch.

Another embodiment of the present invention provides an ungrounded type flexible fabric container with a reduced energy of electrostatic discharge for use in a combustible environment. The container comprises a woven fabric configured to from the flexible fabric container having side walls, a closed end and an open end. The container is made from static dissipating fabric comprising fabric woven of non-conductive tapes of polypropylene, preferably homopolymers, having a melt flow index of 1–6 g/10 min. with a preferred melt flow index of about 3 g/10 min. The tapes have a denier from 500 to 4000 and tape width from 0.07 to 0.40 inches. At any given denier, lower width values result in tapes that are too thick and brittle. This leads to difficulty in weaving. Higher width values lead to tape that is too thin for this application. The tape becomes too wide and leading to problems in drawability and breaks. The fabric may be coated with a layer of molten or extruded polypropylene polymer. The coating is preferably a polypropylene homopolymer with a melt index value of greater than 10 g/10 min. and a preferred value of 10–60 g/10 min. Into the fabric a plurality of strands that dissipate electrostatic charges. The strands are made from conductive staple fibers and are woven into or coated onto the fabric at a spacing of from 3 mm to 100 mm. A preferred spacing is to include a dissipative strand about every inch (25 mm) of the fabric. When woven into the fabric, the dissipative strands are introduced at the time of weaving the fabric.

Although the present invention has been described in terms of specific embodiments, various substitutions of materials and conditions can be made as will be known to those skilled in the art. For example, other polyolefin materials may be used for the non-conductive tapes of the fabric. Other variations will be apparent to those skilled in the art and are meant to be included herein. The scope of the invention is only to be limited by the claims set forth below.

## Other References

1. "Testing the Suitability of FIBCs for Use in Flammable Atmospheres", Vahid Ebadat, James C. Mulligan, *Process Safety Progress*, Vol. 15, No. 3, AIChE.
2. Temporary PRODUCT SPECIFICATION for NOSHOCK® CONDUCTIVE FIBER/STAPLE BLEND 285-ES3, October 2000, Solutia, Inc.
3. Prototype FIBC test results from Chilworth Technology dated Sep. 14, 2000
4. Prototype fabric test results from Institute of Safety & Security Test Report 200664.01.5050.

What is claimed is:

1. A static dissipating fabric providing reduced energy of electrostatic discharge for use in a combustible environment without the need for antistatic coatings comprising fabric woven of non-conductive tapes, to which a plurality of antistatic yarn segments are woven into or coated onto the fabric at a spacing of from 3 mm to 100 mm and wherein the antistatic yarn segments comprise yarn segments of conductive and non-conductive staple fibers and wherein the conductive staple fibers are fibers having a conductive constituent on an outer surface of a non-conductive constituent and wherein the conductive constituent is formed into one or more longitudinal stripes.

2. The static dissipating fabric of claim 1 wherein the polypropylene fabric further comprises 11 of 900 denier tapes/inch in the warp direction and 9 of 1300 denier tapes/inch in the weft direction;

wherein tapes further comprise polypropylene homopolymer with ultraviolet inhibitors.

3. The static dissipating fabric of claim 2 wherein the conductive staple yarn is woven into the fabric at a spacing from 10 mm to 100 mm.

4. The static dissipating fabric of claim 2 wherein the conductive staple yarn is woven into the fabric at a spacing of 25 mm.

5. The static dissipating fabric of claim 2 further comprising a polymeric coating.

6. The static dissipating fabric of claim 5 wherein the polymeric coating comprises 79.5% weight polypropylene homopolymer; 19% weight low density polyethylene polymer and 1.5% weight ultraviolet inhibitors.

7. The static dissipating fabric of claim 6 wherein the conductive staple yarn is woven into the fabric at a spacing from 10 mm to 100 mm.

8. The static dissipating fabric of claim 6 wherein the conductive staple yarn is woven into the fabric at a spacing of 25 mm.

9. The static dissipating fabric of claim 5 wherein the polymeric coating comprises 73.5% weight polypropylene homopolymer; 19% weight low density polyethylene polymer; 1.5% weight ultraviolet inhibitors and 6% weight of 25% weight antistatic masterbatch.

10. The static dissipating fabric of claim 9 wherein the conductive staple yarn is woven into the fabric at a spacing from 10 mm to 100 mm.

11. The static dissipating fabric of claim 9 wherein the conductive staple yarn is woven into the fabric at a spacing of 25 mm.

12. A static dissipating fabric providing reduced energy of electrostatic discharge for use in a combustible environment without the need for antistatic coatings comprising fabric woven of non-conductive tapes, to which a plurality of antistatic yarn segments are woven into or coated onto the fabric at a spacing of from 3 mm to 100 mm and wherein the antistatic yarn segments comprise yarn segments of conductive and non-conductive staple fibers and wherein the conductive staple fibers comprise a bicomponent conductive staple fiber having 1 or more longitudinal stripes of a carbon loaded conductive constituent and wherein the conductive staple fibers are fibers having a conductive constituent on an outer surface of a non-conductive constituent and wherein the conductive constituent is formed into one or more longitudinal stripes.

13. The static dissipating fabric of claim 12 wherein the polypropylene fabric further comprises 11 of 900 denier tapes/inch in the warp direction and 9 of 1300 denier tapes/inch in the weft direction;

wherein tapes further comprise polypropylene homopolymer with ultraviolet inhibitors.

14. The static dissipating fabric of claim 12 wherein the antistatic yarn segments comprise 50% by weight non-conductive staple fibers and 50% by weight conductive staple fibers.

15. The static dissipating fabric of claim 13 wherein the conductive staple yarn is woven into the fabric at a spacing from 10 mm to 100 mm.

16. The static dissipating fabric of claim 13 wherein the conductive staple yarn is woven into the fabric at a spacing of 25 mm.

17. The static dissipating fabric of claim 13 further comprising a polymeric coating.

18. The static dissipating fabric of claim 17 wherein the polymeric coating comprises 79.5% weight polypropylene homopolymer; 19% weight low density polyethylene polymer and 1.5% weight ultraviolet inhibitors.

19. The static dissipating fabric of claim 18 wherein the conductive staple yarn is woven into the fabric at a spacing from 10 mm to 100 mm.

20. The static dissipating fabric of claim 18 wherein the conductive staple yarn is woven into the fabric at a spacing of 25 mm.

21. The static dissipating fabric of claim 17 wherein the polymeric coating comprises 73.5% weight polypropylene homopolymer; 19% weight low density polyethylene polymer; 1.5% weight ultraviolet inhibitors and 6% weight of 25% weight antistatic masterbatch.

22. The static dissipating fabric of claim 21 wherein the conductive staple yarn is woven into the fabric at a spacing from 10 mm to 100 mm.

23. The static dissipating fabric of claim 21 wherein the conductive staple yarn is woven into the fabric at a spacing of 25 mm.